

# UNITED STATES PATENT OFFICE.

FLOYD J. METZGER, OF NEW YORK, N. Y., ASSIGNOR TO AIR REDUCTION COMPANY,  
OF NEW YORK, N. Y., A CORPORATION OF NEW YORK.

## RETORE.

1,422,878.

Specification of Letters Patent. Patented July 18, 1922.

No Drawing.

Application filed October 11, 1917. Serial No. 195,951.

To all whom it may concern:

Be it known that I, FLOYD J. METZGER, a citizen of the United States, residing in New York, county of New York, State of New York, have invented certain new and useful Improvements in Retorts, of which the following is a specification.

In many manufacturing operations where retorts, furnaces and the like are subjected to a high temperature it is desirable to employ iron or other similar relatively cheap and plentiful metal as the retort or furnace material. For example, in the manufacture of coal gas, oil gases and in certain processes employed to effect the fixation of atmospheric nitrogen and in numerous other processes not necessary to be mentioned, iron retorts or furnaces would be highly desirable were it not for the fact that the corrosion or oxidation of the retort or furnace is quite rapid at the rather high temperatures required in these processes. The rapid deterioration and destruction of retorts or furnaces consisting of iron or other similar metal involves in many cases a prohibitive maintenance cost and a consequent or necessary elimination of iron as a furnace material for such purposes.

I have discovered that by properly treating the iron; that is, by providing it with a coating of material which is practically unaffected by or which offers substantial resistance to the corrosive or oxidizing action of the gases which are generated in a retort or furnace, I am enabled to protect such iron or other similar suitable metal to a very great extent if not entirely against the corrosive action of such gases. As a result the life of the retort or furnace is greatly prolonged, thereby reducing the up-keep expense of the same to a point at which the use of iron and such other similar metals as may be found to be practicably suitable for retort or furnace material becomes commercially feasible.

My invention comprehends the idea that all parts of the surface of the retort or furnace with which the retort or furnace gases contact shall be coated over in a proper manner with a metal or metal alloy which offers substantial resistance to the corrosive or oxidizing action of the retort or furnace gases.

I have found that an alloy of nickel and chromium in the proper proportions with or

without the addition of relative small quantities of other metals serves very well as such a protective coating for a retort or furnace of iron.

The principal object of my invention is to provide the iron or other similar corrodible material which may be employed for the construction of retorts or furnaces to be employed for the purposes previously stated with a coating of metal which will offer substantial resistance to the corrosive action of the retort or furnace gases, such coating to be applied directly to and intimately combined with the portions of the surface of the iron of the retort which, but for the presence of the coating, would be acted upon by the said gases.

I have discovered that an alloy of nickel and chromium in the proper proportions with or without the addition of smaller quantities of other metals serves very well as a protective coating for an iron retort or furnace. Such alloy may consist of 85% nickel and from 10 to 15% chromium, the variations in the latter depending upon the amount of impurities which may be present such, for example, as iron, manganese and carbon. I have also found that an alloy consisting of approximately 50 to 60% of nickel, 10 to 20% of chromium and 10 to 30% of iron may be employed. Such alloys as the foregoing offer substantial resistance to the corrosive or oxidizing action of the retort or furnace gases.

I propose to form the coating of the character above described upon the iron or similar metal of the retort by projecting the coating material in the form of very finely divided or atomic-like particles with great force against the surface to be coated. These particles may be in a molten state and sprayed by means of any known form of atomizing device against the surface to be coated or the said coating metal may be converted in any suitable manner into fine particles and propelled with such speed and force against the surface to be coated that upon the striking of the particles against the surface to be coated the kinetic energy is converted partly into mechanical work and partly into heat so that the finely divided particles are not only intimately combined and connected with the surface portions of the metal of the retort to be coated but the particles themselves are overlapped, inter-

mingled, and welded together so that a uniform, dense and compact coating upon the surface of the iron retort is produced.

This coating in effect practically is integral with the iron or other metal of which the retort is constructed. The said coating, together with the relatively heavy sheet metal to which it is applied may be regarded and considered as a single integral metallic sheet.

The combining of the minute particles of an alloy comprising nickel and chromium with each other and with the iron or other similar metal of the retort provides a novel article of commerce; viz, a retort comprising or consisting of a base metal portion, as iron, and an integral coating of an alloy comprising nickel and chromium as stated. Such an alloy having the characteristic of offering substantial resistance to the corrosive and oxidizing action of the retort or furnace gases and its application as a coating to the required portion or portions of the surface of an iron retort or furnace being feasible I am enabled to employ commercially retorts or furnaces made of iron or

other similar metal which is readily corroded and oxidized by the action of the retort or furnace gases.

I claim:—

1. A retort adapted for use in the manufacture of alkali metal cyanide and to be subjected to the action of oxidizing gases at high temperature, the retort comprising a body of ferrous metal which is corrodible by said gases and a protecting skin coating applied to the outer surface of the body and consisting of a base metal alloy which resists the oxidizing action of said gases.

2. A retort adapted for use in the manufacture of alkali metal cyanide and to be subjected to the action of oxidizing gases at high temperature, the retort comprising a body of ferrous metal which is corrodible by said gases and a protecting skin coating applied to the outer surface of the body and consisting of a nickel-chromium alloy which resists the oxidizing action of said gases.

In testimony that I claim the foregoing as my invention, I have hereunto signed my name this 9 day of October, A. D. 1917.

FLOYD J. METZGER.